# EUROPEAN PATENT SPECIFICATION

(11) **EP 2 733 191 B1**
(45) Date of publication and mention of the grant of the patent: **27.04.2016**
(21) Application number: 13185404.4
(22) Date of filing: 20.09.2013
(51) Int. Cl.: C10M 159/22, C10M 177/00, C10N 10/04, C10N 30/10

(54) **Phenate detergent preparation**
Phenatreinigungsmittelherstellung
Préparation de détergent phénate

(30) Priority: 14.11.2012 EP 12192645
(43) Date of publication of application: 21.05.2014
(73) Proprietor: Infineum International Limited, Abingdon, Oxfordshire OX13 6BB (GB)
(72) Inventor: Delamore, Oliver, Abingdon, Oxfordshire OX13 6BB (GB); Schwaebisch, Dirk, Abingdon, Oxfordshire OX13 6BB (GB); Marsh, Adam, Abingdon, Oxfordshire OX13 6BB (GB)
(74) Representative: Lewis, Pauline Therese

(56) References cited:
- EP-A1- 1 903 093
- US-A- 5 244 588
- US-A- 5 910 468
- US-B1- 6 339 052

## Description

### FIELD OF THE INVENTION

This invention relates to making a sulphurised calcium alkyl phenate detergent and to use of the detergent in internal combustion engine lubrication.

### BACKGROUND OF THE INVENTION

Sulphurised calcium alkyl phenate detergents are well known additive components for internal combustion engine crankcase lubricating oil compositions. However, certain alkylphenol sources (nonylphenol, tetrapropenylphenol) used in their manufacture are classified as reproductive toxins; accordingly, there is a desire to identify other phenol sources.

The art describes a way of meeting this problem. Thus, US-A-5,910,468 ('468) describes the preparation of sulphurised calcium alkyl phenate from, as the phenol source, distilled or hydrogenated-distilled cashew nut shell liquid (CNSL). Distilled CNSL is a mixture of biodegradable meta-hydrocarbyl substituted phenols, where the hydrocarbyl group is linear and unsaturated, including cardanol. Catalytic hydrogenation of distilled CNSL gives rise to a mixture of meta-hydrocarbyl substituted phenols predominantly rich in 3-pentadecylphenol.

A problem with the process described in '468 is to improve the oxidative stability of the sulphurised calcium alkyl phenate detergents thereby produced.

### SUMMARY OF THE INVENTION

The above problem is met according to the invention by using hydrogenated distilled CNSL as the phenol source and by making the phenate in a two-stage process in which the amounts of calcium salt and of promoter are controlled.

The invention provides, in a first aspect, a method of making a sulphurised calcium phenate detergent comprising the stages:
(i) reacting one or more alkyl phenol materials comprising hydrogenated distilled cashew nut shell liquid with first defined amounts of a calcium and of a di- or poly-hydric alcohol, with sulphur in the presence of a solvent; and
(ii) reacting the product of step (i) with second defined amounts of the calcium salt and of the di- or poly-hydric alcohol and carbonating the product;
the total amount of calcium salt and of alcohol being such as to provide a sulphurised calcium phenate of desired TBN; and wherein the first amount of each of the calcium salt and of the alcohol in step (i), relative to its total amount in the method, being less than 50, expressed as a molar percentage; and wherein the molar percentage of the first amount of each of the calcium salt and of the alcohol is not less than 5, expressed as molar percentages of their total amounts.

The invention provides, in a second aspect, a sulphurised calcium phenate detergent obtainable by the method of the first aspect of the invention. The sulphurised calcium phenate detergent has a kinematic viscosity at 100°C of greater than 750 and less than 1200 cSt, preferably greater than 800 to less than 1150 cSt, as measured by ASTM D445.

The invention provides, in a third aspect, a lubricating oil composition comprising, in a major amount, an oil of lubricating viscosity and, in a minor amount, a detergent of the second aspect of the invention.

The invention provides, in a fourth aspect, a lubricating oil composition comprising, in a major amount, an oil of lubricating viscosity and, in a minor amount, a detergent of the second aspect of the invention.

The invention provides, in a fifth aspect, a method of operating an internal combustion engine comprising fuelling the engine and lubricating the engine with the lubricating oil composition of the fourth aspect of the invention.

In this specification, the following words and expressions, if and when used, have the meanings ascribed below:
"Active ingredients" or "(a.i.)" refers to additive material that is not diluent or solvent;
"comprising" or any cognate word specifies the presence of stated features, steps, or integers or components, but does not preclude the presence or addition of one or more other features, steps, integers, components or groups thereof; the expressions "consists of" or "consists essentially of" or cognates may be embraced within "comprises" or cognates, wherein "consists essentially of" permits inclusion of substances not materially affecting the characteristics of the composition to which it applies;
"major amount" means 50 mass % or more of a composition, preferably 60 mass % or more, even more preferably 70 mass % or more;
"minor amount" means less than 50 mass % of a composition, preferably less than 40 mass %, even more preferably less than 30 mass %;
"TBN" means total base number as measured by ASTM D2896.

Furthermore in this specification, if and when used:
"calcium content" is as measured by ASTM D4951;
"phosphorus content" is as measured by ASTM D5185;
"sulphated ash content" is as measured by ASTM D874;
"sulphur content" is as measured by ASTM D2622;
"KV100" means kinematic viscosity at 100°C as measured by ASTM D445.

Also, it will be understood that various components used, essential as well as optimal and customary, may react under conditions of formulation, storage or use and that the invention also provides the product obtainable or obtained as a result of any such reaction.

Further, it is understood that any upper and lower quantity, range and ratio limits set forth herein may be independently combined.

### DETAILED DESCRIPTION OF THE INVENTION

### Method

In the method of the invention, note may be made of the following:

### Calcium salt and alcohol

The calcium salt is preferably calcium oxide or calcium hydroxide. The di- or poly-hydric alcohol, which is also known as the promoter, has the function of phase transferring the calcium from the solid phase into the liquid organic phase and is preferably a 1, 2-vicinal diol, for example ethylene glycol.

The total amount of calcium salt and of alcohol used must be such as to provide a sulphurised calcium phenate of desired TBN. To provide a detergent of improved oxidative stability, the first amounts (i.e. in stage (i)) of each of the calcium salt and of the promoter, relative to their respective total amounts, are less than 50, such as less than 30, such as 20 or less, expressed as molar percentages. Preferably, the first amounts of each of the calcium salt and of the alcohol, expressed as molar percentages of their total amounts, are not less than 10.

### Alkyl phenol materials

A characteristic structural feature of the alkyl phenol materials used in the invention is meta hydrocarbyl-substitution of the aromatic ring where the substituent is attached to the ring at its first (C1) carbon atom. This structural feature is not available by chemical alkyl phenol synthesis such as the Friedel-Crafts reaction of phenol with olefins. The latter typically gives mixtures of ortho and para alkyl phenols (but only around 1% of meta alkyl phenols), and where attachment of the alkyl group to the aromatic ring is at the second (C2) or higher carbon atom.

Cardanol, the product obtained by distilling technical CNSL, typically contains 3-pentadecylphenol (3%); 3-(8-pentadecenyl) phenol (34-36 %); 3-(8, 11-pentadecadienyl) phenol (21-22%); and 3-(8, 11, 14-pentadecatrienyl) phenol (40-41%), plus a small amount of 5-(pentadecyl) resorcinol (c. 10%), also referred to as cardol. Technical CNSL contains mainly cardanol plus some polymerized material. Cardanol may therefore be expressed as containing significant amounts of meta-linear hydrocarbyl substituted phenol, where the hydrocarbyl group has the formula C₁₅H₂₅₋₃₁ and is attached to the aromatic ring at its first carbon atom (C1).

Thus, both cardanol and technical CNSL contain significant quantities of material having long linear unsaturated side chains and only small quantities of material with long linear saturated side chains. The present invention employs material where a major proportion, preferably all of the phenol, contains material with long linear saturated side chains. Such latter material is obtainable by hydrogenating cardanol; a preferred example is 3-(pentadecyl) phenol, where the pentadecyl group is linear and is attached to the aromatic ring at its first carbon atom. It may constitute 50 or more, 60 or more, 70 or more, 80 or more, or 90 or more, mass % of the additive of the invention. It may contain small quantities of 3-(pentadecyl) resorcinol. The invention does not include technical CNSL.

### Carboxylic acid or anhydride (co-surfactant)

The method may be carried out in the presence of a carboxylic acid or anhydride (which is also known as a co-surfactant) such as a long chain carboxylic acid (e.g. stearic acid or lauric acid, oleic acid or alkylsalicylic acid) or the related esters; a long chain carboxylic amide (e.g. tallow amine); a long chain ethoxylated amine; a phenol or alkyl phenol or methylene bridged alkyl phenol; a hydrocarbyl substituted anhydride or succinic anhydride (e.g. polyisobutene succinic anhydride); or a long chain alkylaryl sulphonic acid.

The carboxylic acid or anhydride (co-surfactant) may be present in the range of 1-20, such as 4-12, such as 4-10, such as 4-8, preferably 6-8, mass % based on the total mass of alkyl phenol. Preferably, the carboxylic acid or anhydride (co-surfactant) is provided in step (ii) to avoid the possibility of its adverse interaction with elemental sulphur in step (i).

### Solvent

Process solvents are added to the reaction mixture in order to decrease viscosity of the reaction mixture during synthesis. As is known by those skilled in the art, lowering the viscosity allows improved dispersion of carbon dioxide in the reaction mixture therefore promoting efficient carbonation. These solvents are typically high boiling (>140°C) and unreactive under the conditions used. Examples include isodecanol, cyclohexanol and 2-ethylhexanol.

### Carbonation Temperature

Carbonation is preferably effected at temperatures of greater than 100°C. Carbonation preferably takes place at temperatures from 120 to 210°C, more preferably from 140 to 190°C, most preferably from 150 to 180°C and even most preferably from 160 to 175°C.

### Lubricating Oil Composition

An oil of lubricating viscosity provides a major proportion of the composition and may be any oil suitable for lubricating an internal combustion engine.

It may range in viscosity from light distillate mineral oils to heavy lubricating oils. Generally, the viscosity of the oil ranges from 2 to 40 mm²/sec, as measured at 100°C.

Natural oils include animal oils and vegetable oils (e.g., castor oil, lard oil); liquid petroleum oils and hydrorefined, solvent-treated or acid-treated mineral oils of the paraffinic, naphthenic and mixed paraffinic-naphthenic types. Oils of lubricating viscosity derived from coal or shale also serve as useful base oils.

Synthetic lubricating oils include hydrocarbon oils and halo-substituted hydrocarbon oils such as polymerized and interpolymerized olefins (e.g., polybutylenes, polypropylenes, propylene-isobutylene copolymers, chlorinated polybutylenes, poly(1-hexenes), poly(1-octenes), poly(1-decenes)); alkybenzenes (e.g., dodecylbenzenes, tetradecylbenzenes, dinonylbenzenes, di(2-ethylhexyl)benzenes); polyphenyls (e.g., biphenyls, terphenyls, alkylated polyphenols); and alkylated diphenyl ethers and alkylated diphenyl sulphides and derivative, analogues and homologues thereof.

Alkylene oxide polymers and interpolymers and derivatives thereof where the terminal hydroxyl groups have been modified by esterification, etherification, etc., constitute another class of known synthetic lubricating oils. These are exemplified by polyoxyalkylene polymers prepared by polymerization of ethylene oxide or propylene oxide, and the alkyl and aryl ethers of polyoxyalkylene polymers (e.g., methyl-polyiso-propylene glycol ether having a molecular weight of 1000 or diphenyl ether of poly-ethylene glycol having a molecular weight of 1000 to 1500); and mono- and polycarboxylic esters thereof, for example, the acetic acid esters, mixed C3-C8 fatty acid esters and C13 oxo acid diester of tetraethylene glycol.

Another suitable class of synthetic lubricating oils comprises the esters of dicarboxylic acids (e.g., phthalic acid, succinic acid, alkyl succinic acids and alkenyl succinic acids, maleic acid, azelaic acid, suberic acid, sebacic acid, fumaric acid, adipic acid, linoleic acid dimer, malonic acid, alkylmalonic acids, alkenyl malonic acids) with a variety of alcohols (e.g., butyl alcohol, hexyl alcohol, dodecyl alcohol, 2-ethylhexyl alcohol, ethylene glycol, diethylene glycol monoether, propylene glycol). Specific examples of such esters includes dibutyl adipate, di(2-ethylhexyl) sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, and the complex ester formed by reacting one mole of sebacic acid with two moles oftetraethylene glycol and two moles of 2-ethylhexanoic acid.

Esters useful as synthetic oils also include those made from C5 to C12 monocarboxylic acids and polyols and polyol esters such as neopentyl glycol, trimethylolpropane, pentaerythritol, dipentaerythritol and tripentaerythritol.

Silicon-based oils such as the polyalkyl-, polyaryl-, polyalkoxy- or polyaryloxysilicone oils and silicate oils comprise another useful class of synthetic lubricants; such oils include tetraethyl silicate, tetraisopropyl silicate, tetra-(2-ethylhexyl)silicate, tetra-(4-methyl-2-ethylhexyl)silicate, tetra-(p-tert-butyl-phenyl) silicate, hexa-(4-methyl-2-ethylhexyl)disiloxane, poly(methyl)siloxanes and poly(methylphenyl)siloxanes. Other synthetic lubricating oils include liquid esters of phosphorus-containing acids (e.g., tricresyl phosphate, trioctyl phosphate, diethyl ester of decylphosphonic acid) and polymeric tetrahydrofurans.

Unrefined, refined and re-refined oils can be used in lubricants of the present invention. Unrefined oils are those obtained directly from a natural or synthetic source without further purification treatment. For example, a shale oil obtained directly from retorting operations; petroleum oil obtained directly from distillation; or ester oil obtained directly from esterification and used without further treatment, are unrefined oils. Refined oils are similar to unrefined oils except that the oil is further treated in one or more purification steps to improve one or more properties. Many such purification techniques, such as distillation, solvent extraction, acid or base extraction, filtration and percolation, are known to those skilled in the art. Re-refined oils are obtained by processes similar to those used to provide refined oils but begin with oil that has already been used in service. Such re-refined oils are also known as reclaimed or reprocessed oils and are often subjected to additional processing using techniques for removing spent additives and oil breakdown products.

The American Petroleum Institute (API) publication "Engine Oil Licensing and Certification System", Industry Services Department, Fourteenth Edition, December 1996, Addendum 1, December 1998 categorizes groups of base stocks. As an example of an oil of lubricating viscosity that may be used in a lubricating oil composition of the present invention, there may be mentioned an oil containing 50 mass % or more of a basestock containing greater than or equal to 90 % saturates and less than or equal to 0.03% sulphur or a mixture thereof. Preferably, it contains 60, such as 70, 80 or 90, mass % or more of said basestock or a mixture thereof. The oil of lubricating viscosity may consist or substantially consist of said basestock or a mixture thereof.

Oil of lubricating viscosity may provide 50 mass% or more of the composition. Preferably, it provides 60, such as 70, 80 or 90, mass % or more of the composition.

The lubricating oil composition may, for example, be a marine diesel cylinder lubricant ("MDCL") or a trunk piston engine oil ("TPEO").

### Engines

The phenates of the invention may be used in lubricants for a range of internal combustion engines (spark-ignited or compression-ignited) such as motor vehicle engines and marine engines. Of the latter, there may be mentioned two-stroke marine diesel cross-head engines and marine trunk piston engines.

### EXAMPLES

The present invention is illustrated by but in no way limited to the following examples.

### Preparation of calcium phenate detergent

The general process was as tabulated and described below:

| **Process description** | **Process detail** |
|---|---|
| Sulphurisation temperature | 140-190°C |
| Sulphurisation time | 2-8 hours |
| Carbonation temperature | 160-175°C |
| Carbonation time | 2-10 hours |
| Sulphur source | S₈ |
| Sulphur charge | 0.20 moles S₈ / CNSL molecule |
| | (1.60 moles S / CNSL molecule) |
| Ca salt | CaO |
| TOTAL Ca CHARGE | 1.43 moles |
| (≡CNSL*) | |
| Promoter | ethylene glycol (EG) |
| TOTAL PROMOTER CHARGE | 2.60 moles |
| (=CNSL) | |
| | |
| Promoter addition temperature | 140°C |
| (stage (i)) | |
| CO₂ charge | 125 mole% |
| | (= Ca salt) |
| Oil | 150N mineral oil |
| Oil charged for synthesis | 22 mass% |
| (=CNSL) | |
| Reaction solvent | isodecanol |
| Co-surfactant | stearic acid |

| | |
|---|---|
| (* means with respect to the total hydrogenated CNSL charge, i.e. for each mole of CNSL material used, 1.43 moles of the calcium source were added) | |

### Step (i)

Hydrogenated distilled CNSL (ex Sigma Aldrich, Cardolite Corporation or synthesized from cardanol sourced from various providers) is sulphurised using elemental sulphur (added in one or two steps) in the presence of calcium oxide, solvent and ethylene glycol.

### Step (ii)

Further ethylene glycol, calcium oxide (such as to provide the required TBN), a co-surfactant and CO₂ are added to the reaction mixture of step (i).

The synthesis is completed by vacuum distillation, filtration or centrifugation, and, if necessary, dilution in oil.

The product was filtered, and diluted to the required TBN with base oil if necessary.

A set of calcium phenate detergents was prepared employing various charges of ethylene glycol promoter and of Ca in each of steps (i) and (ii).

### Tests

The above calcium phenate detergents were blended into otherwise identical marine lubricant formulations (each to contain 9.125 mass % of the detergent), which were subjected to the following test.

### Differential Scanning Calorimetry (pDSC) - [European method no: CECL-85-T-99).]

The test method is performed as follows; ramp at 40°C/min from 50°C to 210°C under an atmosphere of air (689kPa (100psi) and zero flow) then hold at that temperature for up to 2 hours. Open Seiko Aluminium pans are used.

This measures oil induction time and indicates oxidative stability: a higher value indicates a better result. The results are set out in the table below.

| **Example** | **% EG and Ca (step (i))** | **% EG and Ca (step (ii))** | **Kinematic Viscosity (cSt) at 100 °C** | **pDSC (mins)** |
|---|---|---|---|---|
| 1 | 30 | 70 | 919 | 93.7 |
| 2 | 50 | 50 | 1084 | 82.8 |
| A (comparative) | 70 | 30 | 707 | 74.5 |
| B (comparative) | 100 | 0 | 346 | 75.3 |

| | | | | |
|---|---|---|---|---|
| • The percentages are molar percentages; equal molar proportions of EG and Ca were present. • Examples 1 and 2 are examples of the invention, and Examples A and B are reference examples that are for comparative purposes only. | | | | |

The results demonstrate that the use of lower amounts of alcohol and calcium in step (i) in Examples 1 and 2 noticeably increased oxidative stability in comparison with the reference examples (A and B) which included greater than 50% of the total alcohol and calcium in step (i).

## Claims

1. A method of making a sulphurised calcium phenate detergent comprising the steps of:
(i) reacting one or more alkyl phenol materials comprising hydrogenated distilled cashew nut shell liquid with first defined amounts of a calcium salt and of a di- or poly-hydric alcohol, with sulphur in the presence of a solvent; and
(ii) reacting the product of step (i) with second defined amounts of the calcium salt and of the di- or poly-hydric alcohol and carbonating the product;
the total amount of calcium salt and of alcohol being such as to provide a sulphurised calcium phenate of desired TBN; and wherein the first amount of each of the calcium salt and of the alcohol in step (i), relative to its total amount in the method, being less than 50, expressed as a molar percentage; and
wherein the molar percentage of the first amount of each of the calcium salt and of the alcohol is not less than 5, expressed as molar percentages of their total amounts.

2. The method of claim 1, wherein step (ii) is carried out in the absence of sulphur.

3. The method of any one of the preceding claims wherein the calcium salt is calcium oxide or calcium hydroxide.

4. The method of any one of the preceding claims wherein the alkyl phenol material comprises 3-pentadecylphenol.

5. The method of any one of the preceding claims carried out in the presence of a carboxylic acid or anhydride.

6. The method of claim 5, wherein the carboxylic acid or anhydride is stearic acid or a polyisobutene succinic anhydride.

7. The method of any one of the preceding claims, wherein the sulphur is elemental sulphur.

8. The method of any one of the preceding claims, wherein the di- or poly-hydric alcohol is a 1,2-vicinal diol.

9. A sulphurised calcium phenate detergent obtainable by the method of any one of claims 1-8, the sulphurised calcium phenate detergent having a kinematic viscosity at 100°C of greater than 750 and less than 1200 cSt, as measured by ASTM D445.

10. Use of the detergent of claim 9 in a marine crankcase lubricant.

11. Use according to claim 9 in a marine crankcase lubricant to improve the oxidative stability of the lubricant as measured using Differential Scanning Calorimetry (pDSC) (European method no. CECEL-85-T-99) in comparison with that of a lubricant containing a detergent made by a single-stage calcium salt addition process.

12. A lubricating oil composition comprising, in a major amount, an oil of lubricating viscosity and, in a minor amount, a detergent of claim 9.

13. The lubricating oil composition of claim 12, wherein the oil of lubricating viscosity contains 50 mass % or more of a basestock containing greater than or equal to 90 % saturates and less than or equal to 0.03 % sulphur or a mixture thereof.

14. The lubricating oil composition of claim 12 or claim 13 in the form of a marine diesel cylinder lubricant.

15. The lubricating oil composition of claim 12 or claim 13 in the form of a marine diesel trunk piston engine oil.

16. A method of operating an internal combustion diesel engine comprising fuelling the engine, and lubricating the engine with a lubricating oil composition of any of claims 12-15.

## Patentansprüche

1. Verfahren zur Herstellung von geschwefeltem Calciumphenat-Detergens, bei dem
(i) ein oder mehrere Alkylphenol-Materialien, die hydrierte destillierte Cashewnußschalenflüssigkeit mit ersten festgelegten Mengen an Calciumsalz und zwei- oder mehrwertigem Alkohol aufweist, mit Schwefel in der Gegenwart von Lösungsmittel umgesetzt wird und
(ii) das Produkt aus Schritt (i) mit zweiten festgelegten Mengen des Calciumsalzes und des zwei- oder mehrwertigen Alkoholes umgesetzt wird und das Produkt carbonisiert wird,
wobei die Gesamtmenge an Calciumsalz und Alkohol so ist, dass ein geschwefeltes Calciumphenat mit gewünschter TBN bereitgestellt wird, und wobei die erste Menge des Calciumsalzes und des Alkoholes in Schritt (i) jeweils bezogen auf ihre Gesamtmenge in dem Verfahren weniger als 50 beträgt, ausgedrückt als Molprozentsatz, und
wobei der Molprozentsatz der ersten Menge des Calciumsalzes und des Alkoholes jeweils nicht weniger als 5 beträgt, ausgedrückt als Molprozentsatz ihrer Gesamtmengen.

2. Verfahren nach Anspruch 1, bei dem Schritt (ii) in der Abwesenheit von Schwefel durchgeführt wird.

3. Verfahren nach einem der vorhergehenden Ansprüche, bei dem das Calciumsalz Calciumoxid oder Calciumhydroxid ist.

4. Verfahren nach einem der vorhergehenden Ansprüche, bei dem das Alkylphenol-Material 3-Pentadecylphenol umfasst.

5. Verfahren nach einem der vorhergehenden Ansprüche, welches Verfahren in der Gegenwart von Carbonsäure oder -anhydrid durchgeführt wird.

6. Verfahren nach Anspruch 5, bei dem die Carbonsäure oder das Carbonsäureanhydrid Stearinsäure oder Polyisobutenbernsteinsäureanhydrid ist.

7. Verfahren nach einem der vorhergehenden Ansprüche, bei dem der Schwefel elementarer Schwefel ist.

8. Verfahren nach einem der vorhergehenden Ansprüche, bei dem der zwei- oder mehrwertige Alkohol 1,2-vicinales Diol ist.

9. Geschwefeltes Calciumphenat-Detergens, das durch das Verfahren gemäß eines der Ansprüche 1 bis 8 erhältlich ist, wobei das geschwefelte Calciumphenat-Detergens eine kinematische Viskosität bei 100 °C von mehr als 750 und weniger als 1200 cSt aufweist, gemessen gemäß ASTM D445.

10. Verwendung des Detergens gemäß Anspruch 9 in Schiffskurbelwannen-Schmiermittel.

11. Verwendung nach Anspruch 10 in Schiffskurbelwannen-Schmiermittel, um die oxidative Stabilität des Schmiermittels, gemessen unter Verwendung Dynamischer Differenzkalorimetrie (pDSC) (Europäische Methode Nr. CECL-85-T-99), im Vergleich zu der eines Schmiermittels zu verbessern, das ein Detergens enthält, das in einem einstufigen Calciumsalz-Zugabeverfahren hergestellt worden ist.

12. Schmierölzusammensetzung, die in einer größeren Menge Öl mit Schmierviskosität und in einer kleineren Menge Detergens gemäß Anspruch 9 umfasst.

13. Schmierölzusammensetzung nach Anspruch 12, bei der das Öl mit Schmierviskosität 50 Massen-% oder mehr Basismaterial enthält, das mehr als oder gleich 90% gesättigte Materialien und weniger als oder gleich 0,03% Schwefel oder eine Mischung davon enthält.

14. Schmierölzusammensetzung nach Anspruch 12 oder 13 in der Form von Schiffsdieselzylinder-Schmiermittel.

15. Schmierölzusammensetzung nach Anspruch 12 oder 13 in der Form von Schiffsdieseltauchkolbenmotor-Schmiermittel.

16. Verfahren zum Betreiben von einem Dieselverbrennungsmotor, bei dem der Motor angetrieben wird und der Motor mit Schmierölzusammensetzung gemäß eines der Ansprüche 12 bis 15 geschmiert wird.

## Revendications

1. Procédé de préparation d'un détergent à base de phénate de calcium sulfuré, comprenant les étapes de :
(i) réaction d'une ou plusieurs substances du type alkylphénol comprenant du liquide de coquille de noix de cajou distillé hydrogéné avec des premières quantités définies d'un sel de calcium et d'un alcool di- ou polyhydroxylique, avec du soufre en présence d'un solvant ; et
(ii) réaction du produit de l'étape (i) avec des secondes quantités définies du sel de calcium et de l'alcool di- ou poly-hydroxylique et carbonatation du produit ;
la quantité total de sel de calcium et d'alcool étant choisie de manière à fournir un phénate de calcium sulfuré ayant l'indice de basicité total (TBN) désiré ; et dans lequel la première quantité de chacun du sel de calcium et de l'alcool dans l'étape (i), par rapport à leurs quantités totales dans le procédé, est inférieure à 50, exprimée en pourcentage molaire ; et
dans lequel le pourcentage molaire de la première quantité de chacun du sel de calcium et de l'alcool est non inférieure à 5, exprimé en pourcentage molaire de leurs quantités totales.

2. Procédé suivant la revendication 1, dans lequel l'étape (ii) est mise en oeuvre en l'absence de soufre.

3. Procédé suivant l'une quelconque des revendications précédentes, dans lequel le sel de calcium est l'oxyde de calcium ou l'hydroxyde de calcium.

4. Procédé suivant l'une quelconque des revendications précédentes, dans lequel la substance du type alkylphénol consiste en le 3-pentadécylphénol.

5. Procédé suivant l'une quelconque des revendications précédentes, mis en oeuvre en présence d'un acide ou anhydride carboxylique.

6. Procédé suivant la revendication 5, dans lequel l'acide ou anhydride carboxylique est l'acide stéarique ou un anhydride polyisobutène succinique.

7. Procédé suivant l'une quelconque des revendications précédentes, dans lequel le soufre est le soufre élémentaire.

8. Procédé suivant l'une quelconque des revendications précédentes, dans lequel l'alcool di- ou polyhydroxylique est un diol 1,2-vicinal.

9. Détergent à base de phénate de calcium sulfuré pouvant être obtenu par le procédé de l'une quelconque des revendications 1 à 8, le détergent à base de phénate de calcium sulfuré ayant une viscosité cinématique à 100°C supérieure à 750 et inférieure à 1200 cSt, telle que mesurée suivant la norme ASTM D445.

10. Utilisation du détergent de la revendication 9, dans un lubrifiant de carter de moteur marin.

11. Utilisation suivant la revendication 9 dans un lubrifiant de carter de moteur marin pour améliorer la stabilité à l'oxydation du lubrifiant, telle que mesurée par calorimétrie à balayage différentiel (pDSC) (procédé européen n° CECEL-85-T-99) par comparaison avec celle d'un lubrifiant contenant un détergent préparé par un procédé d'addition de sel de calcium en une seule étape.

12. Composition d'huile lubrifiante comprenant, en une quantité dominante, une huile de viscosité propre à la lubrification et, en une petite quantité, un détergent de la revendication 9.

13. Composition d'huile lubrifiante suivant la revendication 12, dans laquelle l'huile de viscosité propre à la lubrification contient 50 % en masse ou plus d'une huile lubrifiante de base contenant une quantité supérieure ou égale à 90 % de composés saturés, et une quantité inférieure ou égale à 0,03 % de soufre ou un de leurs mélanges.

14. Composition d'huile lubrifiante suivant la revendication 12 ou la revendication 13, sous forme d'un lubrifiant de cylindres de moteurs diesel marins.

15. Composition d'huile lubrifiante suivant la revendication 12 ou la revendication 13, sous forme d'une huile de moteurs diesel marins à piston-fourreau.

16. Procédé pour faire fonctionner un moteur diesel à combustion interne, comprenant l'alimentation en carburant du moteur et la lubrification du moteur avec une composition d'huile lubrifiante de l'une quelconque des revendications 12 à 15.
